

Jan. 15, 1935.

R. WEINGAND ET AL  
PROCESS OF INCREASING THE MOISTUREPROOF  
QUALITIES OF SHEETS OF ORGANIC MATTER  
Filed April 21, 1932

1,988,099

Fig.1



Fig.2.

Fig.3.

R. Weingand & J. Seiberlich  
INVENTORS.

by: *Marko Klock*  
ATTY.S.

## UNITED STATES PATENT OFFICE

1,988,099

PROCESS OF INCREASING THE MOISTURE-  
PROOF QUALITIES OF SHEETS OF OR-  
GANIC MATTERRichard Weingand and Josef Seiberlich, Bomlitz,  
near Walsrode, GermanyApplication April 21, 1932, Serial No. 606,717  
In Germany December 29, 1931

2 Claims. (Cl. 91—70)

This invention has reference to the treatment of thin sheets of solidified cellulose solutions and the like by means of which the objectionable effects of the hygroscopic or moisture-reducing qualities of such material are obviated or entirely eliminated and the adaptability of this kind of material is increased and a great improvement in the quality of the product and of the course of manufacture, particularly for 5 a great many industrial and other purposes may be produced. It is well known that all opaque and transparent or translucent foils or thin sheets of plates of cellulose, and of cellulose compounds, as well as sheets and plates of gelatine and the like present the very serious drawback that these articles and products made therefrom on account of their hygroscopic nature are more or less permeable for water vapors and steam. In view of these facts articles and 10 objects which are hygroscopic themselves and which have been wrapped up in foils or sheets of the material referred to are dried up in accordance with the amount of moisture in the atmosphere; or such objects absorb moisture 15 very readily, so that in a great number of cases the wrapped up articles become unfit for use. As instances of such articles and objects various alimentary articles may be mentioned, such as biscuit, crackers, pastry, cakes, sweets, candy, 20 cheese, coffee, tea, tobacco products, hygroscopic salts and many other articles. For shipping and packing purposes of such articles and objects and for storage thereof they will have to be packed or wrapped up, so as to be proof against 25 the action of water vapors.

Various suggestions to overcome this difficulty have been made in the prior art in connection with the wrapping and enclosing means in use. Of these a scheme may be mentioned according 30 to which paper has been impregnated or coated with a layer of oil or of wax; or in accordance with another instance sheets or foils of paper were pasted onto metal foils or thin sheets of metal, for instance in the art of packing or 35 wrapping up crackers and the like. In the case of transparent foils of cellulose-hydrate, ester of cellulose or gelatine it has been suggested to coat foils or sheets thereof with a solution of a cellulose ester in a volatile organic solvent in 40 which resins, waxes and softening agents have also been dissolved, in order to reduce the permeability thereof for water vapors; the varnish film which remains upon the foils or sheets after the evaporation of the solvent produces the 45 desired imperviousness against the action of 50

water vapors. However, the carrying out of this method presents certain difficulties and calls for an extensive, space requiring apparatus, and it is by no means easy to remove the solvents without any residue, inasmuch as this can only be done by an increase of temperature which is liable to impair the quality of the material. Yet, the absolute freedom from solvent is a necessity, because the sheets and foils, particularly in the case of the wrapping up of foods, 5 must be perfectly inodorous. On the other hand, if the solvents are not removed without residue, the aggregated foils or sheets in a pile are likely to become pasted to each other. There is the additional inconvenience that the coating of varnish very often becomes turbid in consequence 10 of the vaporization of the solvents, so that the required glassy clearness of the transparent foils is seriously interfered with. Moreover, this procedure is rather expensive in view of the 15 fact that even with the most careful recovery a portion of the solvent is lost, and the recovery 20 of the solvent necessitates an expensive series of apparatus which consume heat and energy. 25

Now, as a result of lengthy investigations and experiments it has been ascertained that a high degree of impermeability against the action of water vapors at least equal to that of a coating of varnishes of cellulose-esters obtained by the 30 aid of solvents may be produced upon sheets or foils of the kind referred to or upon articles comprising the same without the use of a volatile solvent and in a far more simple and less expensive manner than heretofore by applying the coating material in which cellulose-compound are contained, to the base in the liquid or semi-solid condition instead of preparing a volatile solution thereof. This object is accomplished in our invention by making use of the 35 resins or softening means contained in the coating compound or of a combination of these means as solvents for the cellulose compounds. Such resins and softening means reduce the 40 permeability for water vapors of the coating and they also impart to the cellulose-compound 45 and consequently to the coating the desired pliability and hardness, so as to prevent the peeling off of the varnish otherwise caused by mechanical strains acting upon the foils, sheets or 50

It has also been found to be of advantage to add waxes, wax-like bodies and the like as additional water repelling agents to the coating material in combination with the components above 55 referred to. In a preferred embodiment of the

invention we may proceed by adding and incorporating the cellulose compound with the fused resin slowly and by thorough agitation by which means the cellulose compound becomes dissolved in the resin. Then the further additions, such as softening agents and waxes are added and the mixture is continued to be heated with agitation, until the melt has become homogeneous.

As cellulose compounds which have proved to be suitable for our purposes we may mention the following:—nitro-cellulose, acetyl-cellulose, stearyl-cellulose, palmityl-cellulose, ethyl-cellulose, benzyl-cellulose. Of resins natural and artificial resins are to be used, such as for instance, rosin, dammar-gum or -resin, gum copal and the well known resin-esters. As softening agents we may advantageously make use of all kinds of plasticity imparting agents usually employed in combination with cellulose compounds, such as for instance, camphor, tricresyl-phosphate, triphenyl-phosphate, methyl-cyclohexanol and the like. Additions such as beeswax, ceresine, carnauba-wax, paraffine, vaseline, wool-grease in view of their water repelling properties are well adapted to considerably increase the impermeability for water vapors of the coating material.

The coating which may comprise a solution of a cellulose compound in one or more resins or softening agents with or without the addition of waxes or wax-like bodies may for instance be applied by passing the sheets, foils and the like through the molten mixture, any existing excess being removed by a scraping or similar device. The process may, however, be modified by applying and distributing the molten or semi-solid compound upon the foil or sheet to be coated by means of rotating rollers or brushes, and then smoothening the coat, after it has become solidified, by means of soft brushes. We may also apply the molten material to the surface by means of sprayers or spraying pistols, and then, after solidification, smoothen the coat. For the purpose of more thoroughly attaching the coating layer to the surface the particular sheet or foil may be preheated for a short time. It has also been found to be of advantage for the formation of the coating film of varnish upon the foil to maintain the coating for a short time after application thereof at an increased temperature, and particularly at its melting temperature, by which means the union of the coat with the surface is also assisted. This subsequent heating may be produced for instance by passing the sheets, foils or webs through a heated room or over heated rollers.

In accordance with the intended utilization of the coated article it may be provided with a thin or thick covering layer. It has been ascertained that a film-like layer of one  $\mu$  thickness is already sufficient to impart the desired imperviousness against water-vapors to the sheets. The coating may, of course, be applied to one or both sides of the sheet or foil. Inasmuch as such coatings of the required thickness are perfectly transparent, they are particularly suitable for the reduction of the permeability for water vapors otherwise possessed by transparent sheets, such as thin sheets or foils of cellulose-hydrate, cellulose-compounds, gelatine and polymerization products. Sheets coated in accordance with this invention present the additional advantage that they may be united without the use of adhesives. In carrying out this

feature of our invention the portions of the sheets or foils to be united are placed upon each other and are heated for a short time to about 70 degrees centigrade, which results in the welding together of the contacting surfaces. This modification of the process is particularly of importance for the packing of articles by machinery.

#### Examples

1. Into one kilogram of rosin or colophony heated to 80° C. 100 grams of benzyl-cellulose are introduced with thorough agitation, thereby causing the latter to be dissolved. Thereupon 500 grams of beeswax and 100 grams of tricresyl-phosphate are added to the solution and the mass is stirred at 80° C., until a homogeneous melt has been obtained. This product is applied by a roller brush to an endless web of parchment paper. After the coating has been effected, the web is passed through a drying tunnel or the like which has been heated to 60 degrees C. at a speed to allow the web to remain therein for about 30 seconds. After cooling the web is rolled up.

2. The coating mixture comprises the following constituents:—

100 grams tricresyl-phosphate,  
100 grams nitrocellulose containing 11.5 percent nitrogen,  
500 grams gum dammar,  
400 grams carnauba wax,  
the nitrocellulose being kneaded together with the softening agent and being then worked into a homogeneous melt with the other ingredients at 70 degrees C. The resulting compound is applied in the molten state by means of a spraying pistol to a transparent sheet or foil of cellulose-hydrate, so as to constitute a layer of 0.001 millimeter after the solidification of which it is smoothened by means of a soft brush.

The accompanying drawing shows by way of example several practical embodiments of the invention in Figures 1, 2 and 3 in schematic representation, in which Fig. 1 is a diagrammatic vertical section of the device and Figs. 2 and 3 similar views of modifications.

According to Figure 1 the foil 1 of cellulose hydrate is passed from the roll 4 through the receptacle 2 containing the coating solution 3 and then through the scraping device 5. The foil 1 is coated on its both sides with solution when going through the receptacle 2 and any existing excess of solution will be removed by the scraping device 5 from the foil after leaving the receptacle. The foil is then conducted away over the roll 6 and wound up. According to Figure 2 the foil 1 coming from the roll 4 is coated on one side by means of the rotating brush 7 immersing in the coating mass 8 contained in the container 9 and applying coating mass upon the foil 1. The rotating brush 10 uniformly distributes the applied coating mass upon the foil 1 and then the foil is subjected to the action of heat produced by means of a cylinder 11 into the interior of which vapor is introduced. If desired the coating may be smoothened between the guiding roller 12, 15 by means of the soft rotating brush 13, whereupon the foil 1 is wound upon the roller 14. In Figure 3 the foil 1 coming from the roll 4 is conducted through the electric heating device 16 preheating the foil before it passes between the two spraying squirts 17, 18 applying molten coating mass to both the sides of the foil 1. Then the foil is subjected to the

action of the rotating brushes 19, 20 producing the uniform distribution and the smoothening of the coating mass applied. Thereafter the foil 1 goes through the drying tunnel 21 heated to 5 degrees C. by being traversed by hot air and finally the foil is wound up on the roller 14.

It should be pointed out that various changes may be made within the scope of this invention, as for example different kinds and proportions 10 of the coat producing agents and different kinds of preferably flexible sheets may be used, and other changes may be made, except as otherwise appears from the annexed claims.

We claim:—

15 1. The process of making moisture-proof wrappers which comprises fusing a mixture con-

sisting of cellulose derivative, resin, plasticizer and wax, the cellulose derivative being in a minor proportion as to the resin and wax, and applying the mixture to a structureless foil while in a molten condition.

2. The process of making moisture-proof wrappers which comprises fusing a mixture consisting of cellulose derivative, resin, plasticizer and wax and applying the mixture to a structureless foil while in molten condition, said derivative being approximately in the proportion of 100 parts to 500 parts of said other ingredients.

RICHARD WEINGAND.  
JOSEF SEIBERLICH.

15